

June 4, 1929.

H. P. PARROCK

1,716,181

MANUFACTURE OF ALLOY PIG IRON

Filed Dec. 24, 1926



By *John Boyle*  
Attorney

Patented June 4, 1929.

## UNITED STATES PATENT OFFICE.

HARRY P. PARROCK, OF BROOKLINE, MASSACHUSETTS.

## MANUFACTURE OF ALLOY PIG IRON.

Application filed December 24, 1926. Serial No. 156,799.

My invention relates to a new method of making alloy pig iron. Heretofore pig iron alloys have been made in several different ways. A natural ore containing the alloying metals has been smelted in the blast furnace. One of the best known alloys from an ore of this character contains approximately one per cent nickel and two per cent chromium. The pig iron resulting from this natural ore contains the alloying metals as they naturally occur and the proportions are not subject to correction in the manner in which it is now produced. At the present time no known ores of iron contain all the auxiliary metals now coming into use, such as nickel, chromium, tungsten, vanadium, aluminum, molybdenum and others and no ores contain silicon, phosphorus and manganese in suitable proportions.

In the foundry, an alloy in the form of a ferro alloy is added to the molten iron in the ladle. It is also sometimes charged in the stack. Lacking control of the temperature and being pushed for time to allow the alloy to dissolve and because of the loose methods segregation often occurs. These processes lack exactness and bring variable results.

One of the advantages of my process is that the waste of alloys in the usual and prevailing method of introducing such alloys in foundry practice will be reduced if the alloy has already been made in the pig iron.

One of the objects of my invention is to introduce these auxiliary metals into molten iron in an economical manner. A further object is to provide a means for easily correcting the contents of those auxiliary metals already present, such as manganese, silicon, phosphorous, carbon and sulphur.

Still another object is to provide a practical method of improving the grey iron foundry trade by increasing the range of useful irons by the use of alloys while at the same time, the iron maker is to be afforded a means of protecting himself against the loss in time, money and often in reputation arising from "off-iron". By using my invention, an appreciable curtailment may be had in the grades of ore carried for mixing purposes and with consequent reduction in investment and better regulation of practice.

In carrying out my invention, I use an auxiliary melting unit comprising an open hearth furnace of suitable design and an electric fur-

nace. The open hearth furnace may be of the tilting or stationary type and the electric melting furnace may be of any conventional type.

Referring now to the drawing for a more complete disclosure of the invention, there is shown, by way of example, a typical lay-out for the manufacture of alloy pig iron using hot metal direct from the blast furnace.

In this plant 1 is the blast furnace, 2 are hot blast stoves and 3 is the stack therefor. Adjacent the blast furnace are tracks 4 on which run slag ladles 5 to receive the slag as it comes down the slag runways 6. On the opposite side of the blast furnace are tracks 7, leading to a pig casting machine, on which run metal ladles 8 to receive the molten metal as it comes down the metal runways 9 from the blast furnace or the runway 10 from the open hearth. The main runway 11 conducts metal into a ladle 12 in the transfer ladle pit 13. Located adjacent the blast furnace is the auxiliary melting unit comprising a regenerative open hearth furnace 14 and an electric melting furnace 15. An overhead crane may run on the track 16 for handling ladles and other materials.

The electric furnace is used to premelt the auxiliary or added alloy, preferably in the ferrous form, as ferro-nickel, with a proportion of the iron coming from the blast furnace, to ensure a perfect alloy. That is, if a bath of twenty-five net tons is to be melted in the open hearth furnace to contain one percent nickel when finished, this one percent or five hundred pounds would be melted as, for instance, one thousand pounds of fifty percent ferro-nickel with one thousand pounds of the molten iron, giving a bath of two thousand pounds in the electric furnace. When the twenty-five ton heat less one thousand pounds have been brought to the proper temperature on the open hearth bottom, the two thousand pounds of ferro-nickel alloy would be transferred from the electric furnace to the open hearth bath.

The open hearth furnace would be fired preferably with coke-oven gas; or it could be fired by oil; or blast furnace gas, or coal gas. A large electric furnace could be used instead of the open hearth, except that the large capacity would entail much more expense. Furthermore, the temperature of the arc is not necessary in this operation. A degree of super-heat above the temperature of the iron determined by the blast furnace may not

always be necessary, since the rich alloy from the electric furnace can be made very hot. But the ability to super-heat the bath of iron is made available by the use of the regenerative feature of the open hearth furnace—a desirable feature in the case of "soft iron" which cools rapidly.

Furthermore if it is desired to remelt cold iron, to reclaim it from "off-iron" or for any other reason the open hearth furnace, or equal electric, can handle such iron.

My process gives a flexibility to the blast furnace enabling it to furnish its trade with relatively small proportions of its out-put in "special iron", without going to the heavy expense of special ores, if available, and of "mixed" operating. That is, it can furnish a carload say of fifty tons, out of an otherwise standard day's run of say five hundred tons which might be made a very soft iron, 3.25 silicon, when the ore pile and operating conditions will be regularly delivering No. 2, plain, say 2.00 percent silicon. In like manner it can deliver any commercial alloy 25 in relatively small lots without upsetting the furnace routine.

From the above description it will be seen that I use an open hearth furnace of suitable size and type conveniently placed to take hot 30 metal, with a small complementary electric furnace for melting alloys.

This melting and alloying unit constitutes an intermediate step between the blast furnace and the pig machine, for that part of the 35 furnace output which can be alloyed to advantage, or which can be corrected for silicon, phosphorus, manganese and possibly carbon. In carrying out the process as disclosed, an acid bottom hearth is assumed, and statements are based on the melting practice inherent in that construction. The action of a basic hearth or of a rammed ore hearth, or of a theoretically neutral hearth is recognized as presenting further phases of the problem, 40 but the limiting conditions do not affect the general principles of my invention. While the use of the present mixer is well established as a means of correcting successive taps by averaging the products and of providing an 45 intermediate collecting point, exercising a steady influence on the process, as in both steel plant and foundry practice, the mixer is not a melting or alloying unit. As an auxiliary 50 between furnace and foundry to regulate pro-

duction and to average the mixture or bath 55 towards a standard formula, the mixer served a definite purpose. But for alloying or even for carburizing or controlling silicon, manganese, phosphorus, or sulphur the higher temperature of the regenerative furnace, or 60 its equivalent is necessary. The complementary small electric furnace in which not only the alloy itself, or the commercial ferro-alloy corresponding, but iron amounting to two to five per cent of that charged on the 65 hearth would be melted with the alloy, would make what may be termed the "rich" alloy. Such solution of the alloy, in a relatively 70 large bath at high temperature ensures quick and thorough solution of the alloy in the open hearth heat which in turn may be super-heated above the usual ladle temperature as may be necessary. The resulting alloy iron is of a quality which the foundry man cannot reach with the melting unit and general facilities 75 at his disposal. Furthermore, the waste in alloys in ordinary foundry practice is very high due to spilling, low temperature of the bath, generally the ladle, and the more or less haphazard method of the industry in such 80 matters. In the case of "off iron" the hearth affords a simple means of correction even for iron that has been stacked in the yards from previous bad runs. In the melting of "off 85 irons" and its correction, the use of local scrap presents possibilities of lower costs of mixture.

I claim:

A method of producing pig iron to also make alloyed pig iron as required without 90 disturbing the normal operation of the blast furnace comprising smelting the ore in a blast furnace, transferring a portion of the molten iron to an open hearth furnace, heating the molten iron in the open hearth furnace to a 95 high temperature, separately melting a relatively small quantity of alloying metal, and without further treatment of the produced molten iron adding the said alloy to the body of metal in the open hearth furnace, there- 100 after casting the alloyed pig iron, in the meanwhile casting the undiverted portion of the molten iron from the blast furnace.

In testimony whereof, I have hereunto set my hand at Brookline, Mass., this 20th day of December, 1926.

HARRY P. PARROCK.